

A. E. SYMMES.  
FLOORING AND METHOD OF LAYING SAME.  
APPLICATION FILED SEPT. 10, 1915.

1,193,843.

Patented Aug. 8, 1916.



Witnesses

S. W. Allen  
J. M. Moreland

Inventor  
A. E. Symmes

By  
John W. Vaughan  
A. E. Symmes

# UNITED STATES PATENT OFFICE.

AMERICUS E. SYMMES, OF MONTREAL, QUEBEC, CANADA.

## FLOORING AND METHOD OF LAYING SAME.

1,193,843.

Specification of Letters Patent.

Patented Aug. 8, 1916.

Application filed September 10, 1915. Serial No. 49,992.

To all whom it may concern:

Be it known that I, AMERICUS E. SYMMES, a citizen of the United States, and resident of the city of Montreal, in the Province of Quebec and Dominion of Canada, have invented certain new and useful Improvements in Flooring and Methods of Laying Same, of which the following is a full, clear, and exact description.

10 This invention relates to improvements in floors, and method of laying same, and the object of the invention is to provide a strong and durable crack, vermin and germ proof floor.

15 A further object is to provide a floor which will be absolutely waterproof.

20 A still further object is to provide a terrazzo floor consisting of marble or other stone particles embedded in asphalt.

25 The terrazzo and mosaic floors at present in such general use, which are claimed to be water and germ proof, are not so strictly speaking, as the binding cement is to a certain degree pervious to moisture and therefore equally pervious to germs. The floors are undoubtedly vermin proof, but can only be crack proof where the foundation layer is free from cracks, as there can be obviously no appreciable elasticity in the hard bedding 30 cements used for the stone chips. It has been realized that this susceptibility of cracking could be overcome by using a bedding cement such as asphalt, but this has heretofore been impracticable owing to the 35 fact that in cooking the mixture of asphalt and stone, the asphalt oil would permeate the stone chips, with the result that a floor made of this material would be of an unsightly and muddy brown color.

40 By means of the process hereafter disclosed, I have overcome this great drawback, and an enabled to produce a floor of marble or other stone chips embedded in an asphalt binder, without injuring or altering the natural colors of the stone chips. This result is accomplished by insulating each stone chip with a substance impervious to the asphalt oil and unaffected by the heat of cooking the asphalt.

45 The process of preparing material for laying the floor consists first in submerging the previously screened and cleaned stone chips in a suitable solution of water glass or sodium silicate. The chips are then dried by any suitable means, and when dried, it will be found that each chip is

completely inclosed in a shell of water glass. It is well known that this material, after drying out of its solution, is insoluble and unaffected by almost any known chemical. 60 The dry coated chips are now mixed with asphalt mastic in proportions varying from 45% stone and 55% asphalt to 55% stone and 45% asphalt, and cooked in the well known manner, at a temperature of from 65 300° to 350° Fahrenheit, until the mass reaches the desired consistency, whereupon it is either molded into blocks for storage and future use, or applied directly to the floor base, spread out into a layer of the desired thickness, and compacted and leveled by rolling or tamping or both. When the asphalt has set hard, the surface of the floor is polished off with stones and water 70 in the well known manner, and when finished, the result is the exposure of the white or variously colored marble or stone chips embedded in a black binder. The percentage of stone in the mixture is varied chiefly according to the use to which the finished 75 floor will be subjected, and the desired hardness of same.

80 In laying the floor, the material is laid on in two coats or courses, the lower of which may be thinner and applied at higher temperature, so as to obtain a perfect bond with the under floor, which is usually a concrete slab. In applying the upper course, care is taken to have any joints between the different patches of material occur on lines 85 remote from similar joints in the lower course, so that in the event of a crack being started in either coat, it will not communicate itself through the other coat, as the upper and lower courses bond together perfectly by reason of the nature of the material. This lower course may also be said to act as a buffer between the base floor and the upper coat, so that the upper coat is relieved of stresses incident to contraction 90 and expansion in the base floor, so that the completed floor will be substantially crack-proof at all temperatures ranging from those below zero to approximately 150°. It will thus be seen that the completed floor 95 is a homogeneous mass from lower to upper surface and from wall to wall.

100 Having thus described my invention, what I claim is:

110 1. A floor composed of individually glazed stone chips embedded in an asphalt binder.

2. A floor composed of stone chips individually coated with material impervious to asphalt oils and embedded in an asphalt binder.
5. A floor composed of stone chips individually coated with sodium silicate and embedded in an asphalt binder.
4. A process of making floors and flooring material, which consists in coating stone chips with an insoluble and impervious material, mixing the chips with a binder, and depositing the mixture in suitable form for setting.
15. A process of making floors and flooring material, which consists in covering stone chips with a coating of material impervious to asphalt oil, mixing the chips with asphalt mastic, cooking the mixture, and depositing the mixture in suitable form for cooling and hardening.
20. A process of making floors, and flooring material, which consists in submerging stone chips in a solution of sodium silicate,

drying the chips, mixing the chips with asphalt mastic, cooking the mixture, and finally depositing the mixture in suitable form for cooling and hardening.

7. A process of making floors and flooring material, which consists in submerging stone chips in an aqueous solution of sodium silicate, drying the chips to form a coating on each individual chip impervious to asphalt oil, mixing the chips with asphalt mastic in a proportion of 45% to 55% chips to 55% to 45% asphalt, cooking the mixture at a temperature of from 300° to 350° Fahrenheit, and finally compacting the mixture in suitable form for cooling and hardening.

In witness whereof, I have hereunto set my hand, in presence of two witnesses.

AMERICUS E. SYMMES.

Witnesses:

C. W. TAYLOR,  
G. M. MORELAND.